

## 1

3,269,949

## GREASE COMPOSITION

Arthur C. Borg, Chicago, Ill., assignor to Standard Oil Company, Chicago, Ill., a corporation of Indiana  
No Drawing. Filed Aug. 30, 1963, Ser. No. 305,832  
5 Claims. (Cl. 252—42.1)

This invention relates to improved lubricating metal soap greases and particularly to lithium soap greases.

It has been discovered that the use of about 0.25—10 weight percent, preferably about 1—6 weight percent, of methyl hydrogen silicone fluid in conventional lubricating metal soap greases improves the lubricity and functional properties of such greases. In addition to such improvements, it was unexpectedly found that use of methyl hydrogen silicone fluid improves the grease yield and its high temperature stability. While the prior art suggests that methyl hydrogen silicone fluid can be used as a lubricant or as a vehicle for grease under non-oxidizing conditions, the discovery that such fluids in the lubricating oil viscosity range, when used in small amounts, in metal soap greases under oxidizing service conditions would act as a lubricity improver was quite surprising and unexpected and in no way predictable.

Lubricating metal soap greases are well known in the art. Such greases are formed by thickening lubricating oil vehicles with metal soaps as the thickening agents. Such metal soaps are the alkali metal and the alkaline earth soaps or unsaturated, partially unsaturated, or saturated fats or fatty acids or hydroxy fatty acids derived from animal, vegetable or marine sources. A fatty acid constituent of such soaps has at least 12 carbon atoms, and preferably from about 12 to 22 carbon atoms. Exemplary of the fatty acids used in preparing metal soap thickening agents are the lauric, myristic, palmitic, stearic, behenic, oleic, hydroxy-stearic, acids, as well as the hydrogenated fish oil fatty acids, hydrogenated castor oil, and mixtures thereof. Exemplary metal soaps are lithium stearate, lithium 12-hydroxy stearate, sodium stearate, barium stearate, strontium soap of hydrogenation fish oil fatty acids, barium-12-hydroxy stearates, calcium soap of hydrogenated castor oil, potassium stearate, etc. Mixtures of such soaps can also be used.

Lubricating oil vehicles that are used in preparing metal soap greases can be petroleum oils in the lubricating oil viscosity range, i.e., from about 25 SSU at 100° F. to about 300 SSU at 310° F. or synthetic hydrocarbon oils such as are obtained by the polymerization of unsaturated hydrocarbons. Other oleaginous materials within the lubricating oil range can be used, such as, for example high molecular weight polyoxyalkylene compounds such as polyalkylene glycol and esters thereof; aliphatic diesters of dicarboxylic acids such as the butyl, hexyl, ethyl hexyl, decyl, lauryl, etc. esters of sebacic acid, adipic acid, azellic acid, etc.; polyfluoro derivatives of organic compounds, particularly hydrocarbons, such as trifluorovinyl chloride polymer, trifluorochloroethylene polymer, etc.

The term "methyl hydrogen silicone fluid" as used herein and in the claims refers to the liquid methyl hydrogen siloxane polymers in the lubricating oil viscosity range. Such polymers are represented by the formula



wherein  $n$  represents an integer that is sufficient for such polymers to have a viscosity in the lubricating oil vis-

## 2

cosity range, namely, of about 25—3500 SSU at 100° F., preferably of about 100—1250 SSU. Such polymers and their preparation are fully described in U.S. 2,491,843.

Illustrative of the improved soap greases of the present invention are multi-purpose lithium soap greases. Such greases are prepared by conventional procedures by the use of from about 5—25 weight percent of a lithium soap, as a thickening agent, in a lubricating oil. For example, a solvent-extracted SAE 40 grade petroleum oil was thickened to grease consistency with 8 weight percent lithium soap obtained from the neutralization of a mixture of hydrogenated castor oil and hydrogenated fish oil fatty acids with lithium hydroxide. This grease had a Timken value of 15 pounds and an ASTM penetration of 304. To a portion of this grease was added 1 weight percent of methyl hydrogen silicone fluid (GE 398-72-857 having a viscosity of about 90 SSU at 100° F., a viscosity index of about 200, a pour point of less than —80° F., and a specific gravity of 1.0050 at 25° C.). After milling, the finished grease containing the methyl hydrogen silicone fluid had a Timken value of 25 pounds, an ASTM penetration of 294 and improved thermal stability at 200° F. The improvement in the Timken value and the reduction in the ASTM penetration value of the lithium soap grease obtained by the addition of the methyl hydrogen silicone fluid illustrates the substantial improvement obtainable by the use of methyl hydrogen silicone fluid. The increase in the Timken value shows that the load-bearing property of such greases is substantially improved. The reduced ASTM penetration value shows that the inclusion of methyl hydrogen silicone fluid in a soap grease produces a harder grease. Consequently, it is possible to obtain a greater yield per pound of thickener.

It will be apparent to one skilled in the art that methyl hydrogen silicone fluid is a very effective lubricity improver and yield improver additive for conventional lubricating metal soap greases.

It is to be understood that the greases of the present invention can contain added constituents such as antioxidants, oiliness agents, extreme pressure additives, anti-foam agents, etc., without in any way departing from the scope of the invention.

I claim:

1. The lubricating grease composition consisting essentially of (A) a hydrocarbon lubricating oil; (B) about 5—25 weight percent of a fatty acid metal soap thickening agent; and (C) about 0.25—10 weight percent of a methyl hydrogen silicone fluid in the lubricating oil viscosity range.
2. The grease composition of claim 1 wherein said lubricating oil is petroleum lubricating oil.
3. The grease composition of claim 2 wherein said metal soap is a lithium soap.
4. The grease composition of claim 3 wherein said lithium soap is derived from a mixture of hydrogenated castor oil fatty acids and hydrogenated fish oil fatty acids.
5. The grease composition of claim 4 wherein the amount of said silicone fluid is about 1—6 percent.

## References Cited by the Examiner

## UNITED STATES PATENTS

- 2,491,843 12/1949 Wilcock ----- 252—49.6  
3,145,175 8/1964 Wright ----- 252—42.1

## FOREIGN PATENTS

- 926,700 5/1963 Great Britain.

DANIEL E. WYMAN, Primary Examiner.

I. VAUGHN, Assistant Examiner.